

## UNITED STATES PATENT OFFICE

2,079,147

## METHOD OF TREATING PELLICLES

Thomas F. Banigan, Kenmore, N. Y., assignor, by  
mesne assignments, to E. I. du Pont de Nemours  
& Company, Wilmington, Del., a corporation  
of Delaware

No Drawing. Application July 28, 1934,  
Serial No. 737,428

8 Claims. (Cl. 215—38)

This invention relates to the prevention of 5  
iron stains, and in particular, it pertains to the  
treatment of pellicles of non-fibrous character,  
such as those made from regenerated cellulose,  
which are adapted for use as bottle caps, bands  
and the like, in order to prevent staining of the  
pellicles when dried in contact with iron or metals  
containing iron as a component.

Heretofore, when regenerated cellulose caps  
10 and bands in a gel condition, i. e. after coagula-  
tion and regeneration but before being dried, were  
applied to bottles having iron-containing metal-  
lic caps or appurtenances, a common defect has  
been that the cellulose caps and bands developed  
15 rust stains which appeared on the surface and  
greatly injured the appearance of the finished  
package. In addition, the portion stained with  
rust became weakened and tended to crack at  
these points.

Caps and bands of regenerated cellulose, which  
20 have been manufactured, for instance, by the  
viscose process, are customarily stored and  
shipped to consumers in an aqueous solution con-  
taining glycerin or other softener. The con-  
sumer withdraws the cap or band from the ship-  
25 ping solution and applies it over the bottle or  
other desired container or object and allows it  
to dry. In drying, it shrinks considerably and  
grips the object tightly. If, in so doing, the cap  
or band comes into contact with iron or metal  
30 containing iron, rust stains will develop, which  
impart an unsightly appearance and a destruc-  
tive action to the cap or band. When the cap  
or band is opaque, as for example when it con-  
tains titanium oxide or other pigment as an  
35 opaquin agent, the unsightliness due to the iron  
stain is quite pronounced.

It is an object of this invention to produce  
non-fibrous pellicles which resist staining when  
40 in contact with iron-containing metals. It is a  
further object of this invention to prevent iron  
stains in caps and bands of non-fibrous sheet  
materials which are applied in a gel state to bot-  
tles or other containers having iron-containing  
45 metal caps or appurtenances, and which caps and  
bands attain their ultimate condition as the result  
of shrinkage through the loss of moisture. Other  
objects of the invention will appear hereinafter.

The objects of this invention are accomplished,  
50 in the preferred form, by shipping the covering  
material in an aqueous solution containing a  
small amount of a stain-preventative material of  
the type herein described.

I have discovered that iron stains can be greatly  
55 diminished and even completely prevented by

using gel cellulosic pellicles which have been  
treated with a solution of a compound which in-  
hibits the formation and/or absorption of soluble  
iron compounds. In applying the principles of  
the invention, the gel pellicles are immersed in  
5 an aqueous solution of the stain-preventing com-  
pound and the immersion is continued until equi-  
librium is established between the solution and  
the pellicles. It is customary to ship gel regen-  
erated cellulose bottle caps and bands in a dilute  
10 aqueous glycerin solution, the glycerin acting as  
a softener. The caps may be placed in the ship-  
ping container and the treating solution contain-  
ing the desired amount of glycerin and stain-  
inhibitor, then poured in until it covers the pel-  
licles, after which the container may be closed  
15 and shipped, and the treated caps, whenever de-  
sired, placed on the bottles or like vessels, and  
permitted to dry and shrink over the tops of  
the bottles.

Those compounds found to be effective in pre-  
venting iron-staining of pellicles of the character  
described herein are water-soluble compounds  
yielding an alkaline reaction in aqueous solution.  
The alkalinity of these compounds is somewhat  
less than that of a sodium hydroxide solution of  
20 equal concentration, and is not so great as to  
injure the cellulosic pellicle during storage in a  
shipping container or when in place on a bottle.  
Preferred compounds of this character which  
25 operate to prevent iron-staining of cellulosic pel-  
licles are tri-sodium phosphate ( $Na_3PO_4$ ), sodium  
pyrophosphate and triethanolamine. The scope  
of the invention includes the corresponding phos-  
phates of the other alkali metals, e. g. potassium,  
30 and includes also other water-soluble salts which  
give a similar alkaline reaction in water solution  
such as borates and silicates of sodium and potas-  
sium. The scope of the invention also includes  
35 water-soluble amines other than triethanolamine.

The compounds used in accordance with the  
present invention need only to be soluble in water  
to the extent desired to inhibit iron-staining, e. g.  
so as to form a concentration ordinarily not less  
than about one-half per cent. Compounds which  
45 would otherwise be suitable but which have a  
too high or a too low pH, when dissolved in aque-  
ous solution, may sometimes be used by adding  
buffer materials so that the final pH may be regu-  
lated within the desired limits, for example, to  
50 obtain a final pH corresponding to that of an  
aqueous solution of tri-sodium phosphate.

The following illustrative examples describe  
modes of applying the invention:

Example I.—Gel caps and/or bands of regen-

erated cellulose prepared from viscose and adapted to be applied to bottle tops and necks are packed in a shipping container containing glycerin and tri-sodium phosphate, in such a concentration that, after equilibrium with the moisture in the caps is reached, the shipping solution contains about 5% of glycerin and about  $\frac{1}{2}\%$  of tri-sodium phosphate.

Example II.—The same procedure is followed 10 as in Example I except that the solution, when equilibrium has been reached, contains one to three per cent of sodium pyrophosphate. The caps and bands, when dried as in Example I, are almost completely free from rust stains after long 15 periods of usage.

Example III.—The same procedure is followed 20 as in Example I, except that the equilibrium solution contains 0.2% triethanolamine.

Caps and bands treated in accordance with the 25 preceding examples, when dried down over iron or iron-containing metal bottle caps, even when the latter are filed down to expose the bare metal, remain completely free from rust stains even after a long period of time.

25 The proportion of anti-staining compounds present in the equilibrium solution which is used to ship the pellicles may vary from a fraction of a percent up to the limit of solubility of the compound in the solution. For most practical 30 purposes, the equilibrium solution will contain from one-tenth per cent to five per cent of said compound.

The invention, in its preferred form, applies 35 to the treatment of regenerated cellulose pellicles obtained from viscose, but it may also be applied to regenerated cellulose pellicles obtained from cuprammonium cellulose solution, or to the treatment of cellulose esters such as cellulose acetate, or to cellulose ethers such as ethyl cellulose or 40 glycol cellulose which have been cast in water solution, or to pellicles of gelatin, casein and related substances. The invention may be applied wherein any such pellicles come in contact with iron under conditions where iron-staining might 45 take place in a manner similar to that explained in connection with gel regenerated cellulose caps and bands.

While the invention is preferably applied to gel 50 pellicles, it will be understood that the scope of the invention includes the treatment of pellicles which have been dried and then rewetted prior to treatment.

Moreover, it is to be understood that instead 55 of shipping pellicles submerged in a shipping solution, they may, of course, be removed from

a shipping solution which has attained equilibrium and shipped in a moist condition to the point of use.

Any variation or modification which conforms 5 to the spirit of the invention is intended to be included within the scope of the claims.

I claim:

1. The method which comprises treating non-fibrous cellulosic pellicles which are subject to shrinking by loss of water and which are subject 10 to staining when shrunk in contact with iron with an aqueous solution of a salt which reacts alkaline in water solution and which will inhibit the formation of an iron compound which will discolor said pellicles. 15

2. The method which comprises treating non-fibrous cellulosic pellicles which are subject to shrinking by loss of water and which are subject 20 to staining when shrunk in contact with iron with an aqueous solution of an alkali metal phosphate.

3. The method which comprises treating non-fibrous cellulosic pellicles which are subject to shrinking by loss of water and which are subject 25 to staining when shrunk in contact with iron with an aqueous solution of sodium triphosphate.

4. The method which comprises treating non-fibrous cellulosic pellicles which are subject to shrinking by loss of water and which are subject 30 to staining when shrunk in contact with iron with an aqueous solution of sodium pyrophosphate.

5. A cellulosic pellicle which is subject to shrinking by loss of water and which is subject 35 to staining when shrunk in contact with iron having associated therewith a colorless salt which reacts alkaline in water and which will inhibit the formation of an iron compound which will discolor said pellicle.

6. A cellulosic pellicle which is subject to 40 shrinking by loss of water and which is subject to staining when shrunk in contact with iron having associated therewith alkali metal phosphate.

7. A cellulosic pellicle which is subject to 45 shrinking by loss of water and which is subject to staining when shrunk in contact with iron having associated therewith sodium tri-phosphate.

8. A cellulosic pellicle which is subject to 50 shrinking by loss of water and which is subject to staining when shrunk in contact with iron having associated therewith sodium pyro-phosphate.

THOMAS F. BANIGAN. 55